

## H. COLLOSEUS.

## PROCESS OF GRANULATING MOLTEN SLAG.

APPLICATION FILED MAR. 16, 1910.

980,606.

Patented Jan. 3, 1911.

2 SHEETS-SHEET 1.



Witnesses:

Witnesses:  
James T. Coggin.  
John H. Barnes

Inventor:

Heinrich Colloseeus  
by L. Ko. Böhm,  
Attorney.

H. COLLOSEUS.  
PROCESS OF GRANULATING MOLTEN SLAG.  
APPLICATION FILED MAR. 18, 1910.

980,606.

Patented Jan. 3, 1911.

2 SHEETS-SHEET 2.



Fig. 2

Witnesses:

James H. Guggin.  
Edmund Murray

Inventor:  
Heinrich Colloseus  
by L. H. Dohm,  
Attorney

# UNITED STATES PATENT OFFICE.

HEINRICH COLLOSEUS, OF BERLIN, GERMANY.

## PROCESS OF GRANULATING MOLTEN SLAG.

980,606.

Specification of Letters Patent. Patented Jan. 3, 1911.

Application filed March 16, 1910. Serial No. 549,605.

*To all whom it may concern:*

Be it known that I, HEINRICH COLLOSEUS, a subject of the King of Prussia, and resident of 27 Regensburgerstrasse, Berlin, German Empire, have invented a new and Improved Process for Granulating Molten Slag, of which the following is a specification.

This invention relates to an improved process for granulating molten slag.

It has already been proposed to cause a stream of molten slag to fall upon a drum rotating at a high speed and provided at its outer circumference with a number of nozzles, through which liquid was sprayed through the stream of molten slag. With this arrangement the nozzle-drum had a double duty to perform, viz. firstly to break up the stream or fluid, and secondly to break up the stream of slag. I have found that a better result is obtained by breaking up the stream of molten slag before it reaches the revolving drum. The slag may be broken up in any well-known manner, for instance by a nozzle; preferably the nozzle for breaking up the stream of slag is arranged behind the flowing slag and above the revolving nozzle-drum, so that a more or less horizontal stream of air, liquid or steam is blown through the stream of slag. With this arrangement the fine division of the slag and partly also its treatment with a solvent may take place at the same point. The nozzle-drum fills the space through which the finely divided slag has passed with the vapor, which may be combined with liquids adapted for the treatment of the slag, such as for example salts in solution, so that the stream of finely divided slag is forced to pass in a regular manner through a layer of such finely divided liquids. In this manner the stream of liquids can be conveniently conducted and easily mingled with the stream of slag to be converted.

The process is carried out in suitable apparatus of which one form is shown in the accompanying drawings in which:

Figure 1 represents an apparatus for granulating molten slag in longitudinal section in the direction of the moving slag, and Fig. 2 is a section on line A, B, of Fig. 1.

Similar letters of reference denote like parts in both figures.

In the drawings *a* represents the revolving nozzle-drum which serves the purpose of

filling the space *c* in which the granulation takes place with finely sprayed liquid. Such liquid, for instance a salt solution, say of sulfate of magnesium is introduced into the interior of the drum by means of pipes *b*, *b*. The molten slag, for instance blast furnace slag is introduced through the channel *d*. Below this channel there is a pipe *e* and a second pipe *f* one of which serves for introducing a stream of steam or liquid while the other serves as a conduit for an air current. Either steam, liquid or air may be used to deflect and disintegrate the current of slag *g* or two of these means or all three of them may be used simultaneously for this purpose.

The nozzle-drum is shown in Fig. 2 partly in section and partly in elevation so that the slots *h* through which the liquid enters are fully shown. The nozzle-drum is rotated by means of the power pulley *i*. To prevent particles of slag from falling onto the shaft of the drum whereby same might be heated and injured conical guards *k*, *k*, are provided and *l* represents a funnel through which obnoxious or injurious gases may escape.

I claim:

1. The process of granulating molten slag consisting in subjecting a stream of molten slag to the action of a nearly horizontally applied current of a fluid which is adapted to break up said slag, and then subjecting the finely divided slag to the action of rotating streams of finely divided liquid.

2. The process of granulating molten slag consisting in subjecting a stream of molten slag to the action of a nearly horizontally applied current of a gaseous fluid which is adapted to break up said slag, and then subjecting the finely divided slag to the action of rotating streams of finely divided liquid.

3. The process of granulating molten slag consisting in subjecting the stream of molten slag to the action of a horizontally applied current of gaseous fluids to break up said slag, and then subjecting the finely divided slag to the action of rotating streams of finely divided salt solution.

In witness whereof I have hereunto set my hand in the presence of two witnesses.

HEINRICH COLLOSEUS.

Witnesses:

WOLDEMAR HAUPT,  
HENRY HASPER.